

# UNITED STATES PATENT OFFICE.

HENRY FORCELLON, OF NEW YORK, N. Y., ASSIGNOR TO ALPHA PRODUCTS COMPANY, INC., A CORPORATION OF NEW YORK.

## PROTECTING SPARKING METAL.

1,396,032.

Specification of Letters Patent.

Patented Nov. 8, 1921.

No Drawing.

Application filed March 27, 1919. Serial No. 285,664.

To all whom it may concern:

Be it known that I, HENRY FORCELLON, a citizen of the United States, and a resident of New York city, in the county of New York and State of New York, have invented certain new and useful Improvements in Protecting Sparking Metal, of which the following is a specification.

My invention relates to improvements in protecting sparking alloys, particularly from the action of moisture and the oxygen of the air. Sparking metal is commonly comprised of an alloy of misch-metall (containing mainly cerium) and iron. While my invention may be used in connection with the various kinds of sparking alloys, I prefer an alloy comprising from 70% to 75% of cerium or misch-metall and from 30% to 25% of iron. The alloy may contain traces of other metals which commonly occur in alloys of this class. I prefer to cast the alloy in the form of slender sticks and to break these up into pieces of suitable size for commercial use, but the alloy may be formed into pieces of suitable size and shape in any suitable manner.

To protect such commercial pieces of sparkling alloy, according to the preferred form of my invention, I take 10 pounds of such pieces, each about 3 m. m. in diameter by about 5 m. m. long (comprising about 22,000 pieces) and put them into an iron vessel with 2 oz. of an hydrocarbon oil known as "Lafayette" packing oil. This oil is a straw colored mineral oil having a flash-point of about 380° C., a fire test of about 430° C. and a viscosity of about 190° measured by the Saybolt viscosimeter at 37° C. The oil originates from the Pennsylvania oil fields. Many other oils may be used particularly the mineral or hydrocarbon oils.

The pieces of sparking metal are heated with the oil in the iron vessel, gradually to a temperature of about 350° C. and kept at about 350° C. for about 15 minutes and then the whole is allowed to cool to about 100° C. The pieces are then taken out and any oil remaining thereon is allowed to evaporate as much as it may. The weight of the metal at the end of the process is about the same as at the beginning.

During the time the oil is kept at 350° C. most of the oil is evaporated or driven

off. I believe the oil is cracked by catalytic action of the metal and deposits on the surface of the pieces a tarry material comprising colloidal carbon which remains on the surface as a dense inert non-metallic coating protecting the metal from the action of moisture and oxygen of the air and at the same time giving the pieces a uniform black appearance without substantially affecting or interfering with the sparking properties of the metal when scratched. Since the coating is non-metallic, it, itself, is not liable to oxidation.

While I have described my improvements in great detail and with respect to the preferred form thereof, I do not desire to be limited to such details or form since many changes and modifications may be made and the invention embodied in widely differing forms without departing from the spirit and scope of my invention in its broader aspects.

What I claim as new and desire to secure by Letters Patent, is:

1. The new article of manufacture comprising a sparking alloy having a dense non-metallic protecting coating on its surface, said coating not substantially affecting the sparking properties of said surface. 80

2. The new article of manufacture comprising a sparking alloy having a dense carbonaceous protecting coating on its surface. 85

3. The new article of manufacture comprising a sparking alloy containing mainly cerium and having a protecting coating on its surface produced by the evaporation and decomposition of oil therefrom, said coating not substantially affecting the sparking properties of said surface. 90

4. The new article of manufacture comprising a sparking alloy containing mainly cerium and having a uniformly black protecting coating produced by the evaporation and decomposition of mineral oil therefrom. 95

5. The process of protecting pieces of sparking alloy which consists in heating the metallic pieces with oil to produce a protecting coating thereon. 100

6. The method of protecting pieces of sparking alloy which consists in treating the pieces with a mineral oil and heat to produce a protecting coating thereon. 105

7. The method of protecting pieces of  
sparking alloy containing mainly cerium,  
which consists in treating the pieces with  
mineral oil and heat to produce a black pro-  
5 tecting coating on the surface of the pieces  
which does not materially affect the spark-  
ing properties thereof.

Signed at New York, in the county of  
New York and State of New York, this 1<sup>st</sup>  
day of March, A. D. 1919.

**HENRY FORCELLON.**

Witnesses:

**ALEXANDER HAMS,**  
**L. D. ULRICH.**